

Sept. 25, 1934.

J. DUARRY-SERRA

1,974,879

PROCESS FOR IMPREGNATING THICK TEXTILE PRODUCTS  
WITH LATEX UNDER GREAT HYDRAULIC PRESSURES  
Filed Sept. 17, 1932



Inventor:  
Juan Duarry-Serra  
by S. Sonae,  
Attorney.

## UNITED STATES PATENT OFFICE

1,974,879

## PROCESS FOR IMPREGNATING THICK TEXTILE PRODUCTS WITH LATEX UNDER GREAT HYDRAULIC PRESSURES

Juan Duarry-Serra, Barcelona, Spain

Application September 17, 1932, Serial No. 633,613  
In Germany January 13, 1932

9 Claims. (Cl. 91—68)

This invention refers to a process for impregnating thick textile products with latex under great hydraulic pressures.

The invention has nothing to do with the impregnation of threads and fabrics with rubber solutions on the basis of organic dissolving agents such as benzol, benzine, carbon tetrachloride etc., and it has nothing in common with the impregnation with latex of textile threads and fine spun materials, which, during the following process of manufacture serve as semi-manufactured goods for the elaboration of various kinds of fabrics, driving belts, etc.

The impregnation of fabrics in closed containers by means of a vacuum and subsequent pressure is known through the Austrian Patent No. 84,510, and the English Patent 316,335, but with these two systems it is not possible to make the latex penetrate right inside the fabric, belt, rope, etc., especially when they are tight and thick, and under no circumstances is this possible when a maximum pressure of 60 pounds to the square inch is used, as in the case of the English patent. Further there is another process disclosed in the German Patent No. 169,401, according to which, with very expensive machines, which form a row of calenders, the fabric is mechanically stretched, opened and heated at the same time. This process, however, cannot be utilized for latex, because, without a high hydraulic pressure the substance would only enter the big openings and pores, but it would not go into the inside of the single threads of the fabric, especially when these are close together. The minimum pressure for this purpose would be 50 atmospheres.

The invention consists in forcing the latex, preferably in a concentrated form, into the textile products under very high pressures ranging between 50 and 800 atmospheres. When such high hydraulic pressures are used, normal latex would give a completely negative result, inasmuch as, owing to the friction which occurs as the substance penetrates the fabric, it would coagulate at once, and make further penetration impossible. First of all, therefore, the latex must be stabilized in order to avoid the coagulation. The process of stabilizing latex to avoid the coagulation resulting from acids is well known, but the special stabilizing to avoid coagulation due to friction during the impregnation is new.

In view of the colloidal condition of the latex, there is the great danger that as a consequence of the high pressure an extremely rapid decomposition may set in, which, under certain circumstances, may cause enormous explosions. There-

fore it is absolutely necessary to prevent this, otherwise it would not be possible to employ the process. For this reason one of the advantages of the invention is that the danger of explosion through the addition of the chemical product in question, is overcome.

When the textile product is impregnated through and through by means of the foregoing process, another difficulty has to be conquered, and the difficulty consists in the extraction of the water which has entered the product. In the case of thin fabrics, threads, etc., this is easily achieved through coagulation and vapourizing, for instance by mechanically applied pressure. When thick textile products have to be treated, however, this process cannot be used, for of course the upper surface coagulates first, when the usual means—acetic acid, alum, chloride of iron etc., are employed, and an impermeable coat of rubber is formed at once on account of which the water is still more completely imprisoned in the interior. When the coagulation takes place exclusively through the action of heat, rather thick rubber coatings are also formed, and on these being broken through the action of the steam inside the tension set up is so great and the temperature so high that both the rubber and the fabric are damaged. In accordance with the process described in the present specification, ammonium carbonate is mixed with the latex, which even at low and harmless temperatures gives off a large amount of gas, and when the mixing has been carried out properly the result is the production of pores inside the fabric. As the pressure exerted by the gas inside rises, the coating of rubber which closes these pores will be torn apart, and the moisture will then be able to escape in the form of water or steam through the canals thus opened up.

By means of the above described process, therefore, it is possible thoroughly to impregnate the thickest textile products with latex under the highest pressures, and also extract all the water from the inside, which was not possible up to the present.

It is well known that in the case of textile products of medium thickness it is possible to impregnate them satisfactorily with rubber by the use of the ordinary rubber solutions, but in this case the highest point of concentration is 10 per cent rubber and the remaining 90 per cent is the solvent. By the use of this process, which precludes the utilization of high pressures, for the reasons already given only a small proportion of rubber can be put into the inside 110

of the fabric. The latex, however, can be concentrated up to the point that it contains up to 75 per cent of rubber, so that by employing the above mentioned process, an amount of pure rubber can be made to enter the fabric, which is many times greater than the amount introduced by the hitherto known process, based on the use of the said solutions.

The present position respecting the impregnation by means of latex in comparison with impregnation with rubber solutions has been made known by the work of Dr. Hauser, from which it is understood that after fifteen different impregnation processes, rubber has not been introduced into the interior of cord threads steeped in latex.

See "Mitteilungen aus dem Arbeitsbereich der Metallgesellschaft A. G., Frankfurt/Main, volume 5, November 1930.

20 The following is a detailed description of the process forming the subject matter of the present application.

#### *Treatment of the latex*

25 Some material must be mixed with the latex which increases its viscosity and also serves as a stabilizing agent, so that when entering the fabric the friction may be reduced to a minimum, and thus the coagulation may be prevented.

30 There are various substances appropriate for this, for example the various kinds of water soluble gums, such as Karaya, Gum arabic, tragacanth, and also the fluid exuded by different kinds of seeds such as linseed etc. However, it has been found that besides this, more especially the sap of certain varieties of cactus plants, both increases the viscosity and also has an excellent stabilizing effect, so that alcohol in small quantities can be added to the latex with this sap, without any coagulation occurring. Among the very numerous kinds of cactus plants those must be eliminated whose sap is acid and therefore have a coagulating effect. There are, however, other kinds of cactus plants, and above all the various families of Indian figs, which are also known by the name of "nopal" and in Spain and Morocco are called "chumberas". These plants, which belong to the genus of "*Nopalea coccinellifera*", have a very rich, completely neutral sap, which gives the viscosity and stability necessary for the object in view. Further, to still more increase the viscosity and stability of the latex, a 20 per cent solution of oils soluble in water can be added. Of all the oils that have been tried for the purpose, the best has proved to be castor oil, and also linseed oil can be added, for it facilitates the drying after the impregnation. While this material is being gradually added to the latex, it is recommended that a little ammonia water be added, so as to avoid the formation of a skin on the upper surface of the latex. Latex prepared in this way will not coagulate even under high pressure and with great friction. A very good formula is the following:

#### Parts

|                                                                                     |    |
|-------------------------------------------------------------------------------------|----|
| Latex with 60 per cent dry rubber                                                   | 80 |
| Sap of the nopal cactus belonging to the genus of " <i>Nopalea coccinellifera</i> " | 15 |
| Castor oil soluble in water                                                         | 5  |
| Linseed oil, raw or boiled                                                          | 5  |
| Ammonia water                                                                       | 1  |

15 To this mixture must then be added the other materials necessary for the vulcanizing, such as

sulphur, oxide of zinc, accelerators and anti-oxidants.

After the latex is completely stabilized and has a high viscosity, still other substances must be added to it, which facilitate the penetration into the threads of the fabric. Such materials are already known, and they are chiefly used in the dyeing of textiles to make the dyes enter the fabric better or to make the colours fast. For this purpose the best substance has been found to be alcohol in a specially prepared form. The alcohol coagulates the latex at once by itself, and to overcome the coagulating effect of the alcohol it must be added to the castor oil soap in a 10% solution. The desired effect, i. e. the facilitating of the penetration of the latex, is, however, fully achieved by means of the alcohol. 5 per cent of this mixture of castor oil soap with alcohol can be added to the latex. This product should not be added to the latex (in the exact quantity required for impregnation) until the last moment, for, if the alcohol is allowed to remain for a long time in contact with the latex, it could, even in this altered form, give rise to coagulation. Further, 3 to 5 per cent ammonia carbonate is added, to secure the formation of pores during the process of drying in connection with the impregnation procedure. Finally, to ensure the avoidance of decomposition under high pressures and as a corresponding precaution against explosions, about 5 per cent silicate of soda (waterglass) is added. When this precaution is taken, as confirmed by tests, even if the pressure exceeds 800 atmospheres no explosion takes place. The following may serve as the complete formula:—

| Parts                                                                            |     |
|----------------------------------------------------------------------------------|-----|
| Latex with 60 per cent dry content                                               | 80  |
| Sap of the nopal cactus belonging to the order " <i>Nopalea coccinellifera</i> " | 15  |
| Castor oil soluble in water                                                      | 5   |
| Ammonia water                                                                    | 3   |
| Alcohol in oil soap                                                              | 5   |
| Silicate of soda (waterglass)                                                    | 6   |
| Linseed oil                                                                      | 6   |
| Ammonia carbonate                                                                | 4   |
| Colloidal sulphur                                                                | 2   |
| Colloidal oxide of zinc                                                          | 6   |
| Piperidine penta methylene di-thiocarbamate                                      | 0.5 |
| Di-thio-carbamate cyclohexylethylamine                                           | 0.5 |
| Diphenylguanidin                                                                 | 0.5 |

The fabrics to be impregnated must be as free from acids as possible. If they may contain acids, as for instance in the case of Esparto grass, it is strongly recommended to wash the products before the impregnation takes place, and to treat them with carbonate of soda.

The drawing shows an installation by means of which impregnation may be carried out in accordance with the foregoing indications:—1 is an impregnating cylinder with strong walls, 2 is a latex container, 3 is the vacuum pump, 4 is a three-way cock, 5 is a throttle valve, 6 and 7 are control valves in the covers of the two containers, 8 is a hydraulic pressure pump, 9 a pressure container with a piston 10, on which the pressure water acts, and there is a piston 11, which exerts pressure on the latex. 12 is the water chamber and 13 is the room for the latex when it is under pressure. 14 is a hollow space produced on account of the difference between the cross sections of the two pistons 10 and 11. 15, 16, 17 and 19 are four shutting-off cocks and 18 is an exhaust cock.

The installation works as follows:—

At the beginning the container 2 is filled with prepared latex, and the container 1 is empty. The material to be impregnated is put into the container 1, the cover is put on and the cocks 5, 7 and 17 are closed, 19 being opened, and then the air is taken out of the container 1 by means of the vacuum pump until the highest possible vacuum is produced. So soon as this has been done, the cock 19 is closed, and communication between the containers 1 and 2 is established by opening the cock 5. The latex thereupon enters the pressure chamber from below and fills it completely, after which the valve 6 in the cover of the container 2 is opened and thus the atmospheric pressure can act on the contents of the container 2. The cock 17 is then opened, and the piston 11 comes under the influence of the pressure water, which enters the intermediate chamber 14 through the valve 15, travelling in a downward direction, and the chamber 13 is filled with latex by suction. Then the valves 5 and 15 are closed, 16 and 18 opened, and pressure is given under the piston 10, whereby the latex enters the container 1 from the chamber 13, the valve 7 being opened, until latex comes out of 7, and this guarantees that there is no more air in container 1. Then valve 7 is closed, and now the pressure inside the container 1 can be increased as much as desired. The pressure will be normally 200 atmospheres, but in the case of very thick and very dense fabrics, for example in the case of thick ship's ropes, the pressure must exceed 800 atmospheres. On the other hand, when very open or loosely woven textiles such as jute soles or Esparto grass are treated, the pressure need not exceed 50 to 60 atmospheres. No textile product, however, can be treated at lower pressures if it is desired to get good results. The temperature during the impregnation process should be preferably between 50 and 60 degrees, because the viscosity of all the components of the mixture is the most satisfactory at these temperatures. The duration of the period during which the products are under pressure depends entirely on the properties and thickness of the products in question, and this must be decided by experience in each case. It may be said, however, by way of information, that braided hemp soles, if subjected to a pressure of 70 atmospheres during 5 to 10 minutes, will be completely impregnated, while ropes of a thickness of 7 cm., subjected to a pressure of 100 atmospheres for a considerable time, cannot be thoroughly impregnated, and even at a pressure of 800 atmospheres they must be subjected to the pressure for half an hour.

During the process of impregnation, the vacuum pump will pump free of air that portion of the container 2 not filled with latex, and when the impregnation has been effected, the latex will be sucked from container 1 into container 2 just as at the beginning.

In connection with the impregnation, the material taken from the container 1 will be subjected to a different treatment according to its nature, though this treatment will always be essentially the same. First by some mechanical means the upper surface will be cleared of the sticky latex preparation adhering to it. According to whether it is a case of particles of the fabric, loose threads or ropes material the cleaning process may be effected by special knives or profiled rollers between which the material continually passes. The single soles must be passed between

the rollers one by one, and the material flattened out. Then the material is heated in order to drive out the water produced as a result of the presence of the ammonium carbonate, and this heating can be carried out according to the nature of the outside of the material. The object, however, is always to secure the production of gas consequent on a moderate degree of heating, whereupon all the inside moisture can escape with the gas. If continuous products such as belts or ropes have to be heated, this is best effected by passing them through an exteriorly heated tube of the appropriate length, so that when the objects in question come out of the opposite end of the pipe the drying process is finished. When small pieces such as soles, have to be treated, these will be carried through the heated tunnel by means of an appropriate transport appliance.

It is advisable to coagulate the surface of the material after the taking off of the first thick coat and before it comes into contact with further apparatus, and this can best be done with alcohol, as compared with all other coagulating agents, because the alcohol completely vapourizes and leaves no traces, whereas the various known acids, when they are used to excess, may adversely affect the finished product due to the deposit they leave.

After the water has been driven out by means of the treatment with ammonium carbonate, the product is extremely porous. So long as water is present in the latex, the latter retains all its stickiness, and through the vapourizing of the water through the opened pores, no temperature will be reached that is appropriate for very quick vulcanization, so experience has demonstrated that immediately after complete expulsion of the water, the latex has not yet vulcanized, and therefore a complete and definite closing of the pores is possible. The closing of the pores is effected by passing the material through two rollers, though it must not pass through too fast. Then the impregnated and dried out product is vulcanized by means of any of the commonly known vulcanizing processes, with the application of the necessary heat.

From the formula above set forth the technical man will see that this may be done at a temperature of less than 100 degrees centigrade.

I claim:

1. Process for impregnating thick and dense textile products with latex, consisting in treating the textile products with latex in a closed container under a pressure exceeding 50 atmospheres, whereby the latex is forced into the products.

2. Process for impregnating thick and dense textile products with latex, comprising: adding to the latex the sap of certain kinds of cactus plants, especially that from the leaves of the plant belonging to the genus of "*Nopalea coccinellifera*", whereby its viscosity is increased and coagulation is prevented; and treating the textile products with the latex in a closed container under a pressure exceeding 50 atmospheres.

3. Process for impregnating thick and dense textile products with latex, comprising: adding the sap of the "*Nopalea coccinellifera*" to the latex, whereby its viscosity is increased and coagulation is prevented; adding castor oil soap to the latex; and treating the textile products with the latex in a closed container under a pressure exceeding 50 atmospheres.

4. Process for impregnating thick and dense

- textile products with latex, comprising: adding the sap of the "*Nopalea coccinellifera*" to the latex, whereby its viscosity is increased and coagulation is prevented; adding alcohol to the latex, whereby the impregnation is rendered more complete; and treating the textile products with the latex in a closed container under a pressure exceeding 50 atmospheres. 5
5. Process for impregnating thick and dense textile products with latex, comprising: adding the sap of the "*Nopalea coccinellifera*" to the latex, whereby its viscosity is increased and coagulation is prevented; adding a mixture of alcohol and castor oil soap to the latex, the alcohol being deprived of its power of coagulating the latex by the admixture with castor oil soap; and treating the textile products with the latex in a closed container under a pressure exceeding 50 atmospheres. 10
10. Process for impregnating thick and dense textile products with latex, consisting in treating the textile products with latex in a closed container under a pressure exceeding 50 atmospheres at a temperature of 50° C. to 70° C., whereby the latex is forced into the products. 15
15. Process for impregnating thick and dense textile products with latex, comprising: adding the sap of the "*Nopalea coccinellifera*" to the latex, whereby its viscosity is increased and coagulation is prevented; adding a mixture of alcohol and castor oil soap to the latex, the alcohol being deprived of its power of coagulating the latex by the admixture with castor oil soap; adding silicate of soda (waterglass) to the latex; and treating the textile products with the latex in a closed container under a pressure exceeding 50 atmospheres. 20
20. Process for impregnating thick and dense textile products with latex, comprising: adding the sap of the "*Nopalea coccinellifera*" to the latex, whereby its viscosity is increased and coagulation is prevented; adding a mixture of alcohol and castor oil soap to the latex, the alcohol being deprived of its power of coagulating the latex by the admixture with castor oil soap; adding silicate of soda (waterglass) to the latex; adding ammonium carbonate to the latex; and treating the textile products with the latex in a closed container under a pressure exceeding 50 atmospheres. 25
25. Process for impregnating thick and dense textile products with latex, comprising: adding the sap of the "*Nopalea coccinellifera*" to the latex, whereby its viscosity is increased and coagulation is prevented; adding a mixture of alcohol and castor oil soap to the latex, the alcohol being deprived of its power of coagulating the latex by the admixture with castor oil soap; adding silicate of soda (waterglass) to the latex; adding ammonium carbonate to the latex; and treating the textile products with the latex in a closed container under a pressure exceeding 50 atmospheres. 30

deprived of its power of coagulating the latex by the admixture with castor oil soap; and treating the textile products with the latex in a closed container under a pressure exceeding 50 atmospheres at a temperature of 50° C. to 70° C. 35

8. Process for impregnating thick and dense textile products with latex, comprising: adding the sap of the "*Nopalea coccinellifera*" to the latex, whereby its viscosity is increased and coagulation is prevented; adding a mixture of alcohol and castor oil soap to the latex, the alcohol being deprived of its power of coagulating the latex by the admixture with castor oil soap; adding silicate of soda (waterglass) to the latex; and treating the textile products with the latex in a closed container under a pressure exceeding 50 atmospheres. 40

9. Process for impregnating thick and dense textile products with latex, comprising: adding the sap of the "*Nopalea coccinellifera*" to the latex, whereby its viscosity is increased and coagulation is prevented; adding a mixture of alcohol and castor oil soap to the latex, the alcohol being deprived of its power of coagulating the latex by the admixture with castor oil soap; adding silicate of soda (waterglass) to the latex; adding ammonium carbonate to the latex; and treating the textile products with the latex in a closed container under a pressure exceeding 50 atmospheres. 45

JUAN DUARRY-SERRA. 50

|    |     |
|----|-----|
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |